

## UNITED STATES PATENT OFFICE

PERCY A. E. ARMSTRONG, OF NEW YORK, N. Y.

## METHOD OF REDUCING AND CONVERTING METALS AND MAKING ALLOYS

No Drawing.

Application filed July 29, 1927. Serial No. 209,396.

The present invention relates to a process for the production of metals and alloys low in carbon and which may be produced low in silicon or aluminum, or with a definitely controlled amount of silicon or aluminum included. The process is particularly adapted to the treatment of the high melting point metals used as alloying ingredients, such as chromium, vanadium, zirconium, titanium, tantalum and uranium.

10 In the manufacture of alloy steels or of high melting point alloys, it is usual to melt down the main ingredient such for example as iron or nickel and add to the refined main 15 ingredient a ferro-alloy of the alloying metal. Where nickel is the main ingredient, the use of the ferro compound may add an undesirable iron content to the finished product and therefore in such a case the alloy may be 20 added as a pure metal.

In some cases, particularly where iron is the main ingredient, the alloy is added in the form of an oxid which is mixed with the charge of iron and melted down together 25 with a reducing agent. If this is done, the accurate composition of the final product is obtained by adding corrective amounts of the ferro-alloy to the melt after an analysis has been made and before pouring. As another alternative, the basic metal is melted 30 and then an oxid of the alloying metal mixed with a reducing agent is thrown on the slagged surface of the molten metal. So much of the alloying metal as is reduced will 35 sink down into the metal of the bath. This latter process is not entirely satisfactory, for it is almost always attendant by large waste, inasmuch as the oxide of the alloying metal is seldom, if ever, entirely reduced; 40 for example, in the case where one seeks to alloy chromium with iron by adding chromite and a reducing agent to the slag covering the bath of molten iron, only from about 50 to 70% of the chromite is reduced and so 45 much reducing agent has to be used, that the reducing agent is carried into the finished product in undesirable quantities. It will also be found that the bath is highly gasified, or wild, and the slag tends to grow to such 50 proportions that it cannot be handled, and a

great amount of heat is wasted keeping the slag fluid. For example, chromite has a metallic chromium content of about 33½% and an iron content of about 14% so that even if all of the metal is reduced the amount of slag will be greater than the amount of metal. Inasmuch as chromite is very refractory and difficult to fuse it will also be found that the reaction will be slow and will demand a very high temperature which will tend to cause the furnace lining to be cut and damaged.

Even where a ferro-alloy is used the process is a slow and expensive one; for example, if ferro-chromium containing about 65% of chromium with low carbon is thrown on the surface of molten iron in sufficient quantity required in a 5-ton melt of a 15% chromium alloy, from 1½ to 2 hours will be needed to melt the ferro-chromium. Such alloys are usually made in an electric furnace and such a bath as described will pick up at least .05% of carbon for each 30 minutes that the arcs are on, so that if one starts with a practically carbon-free iron, the resulting product will have in excess of from 15% to 20% carbon, whereas, in such an alloy it is usually desirable to keep the carbon content below .10%. In the same way, when metallic chromium is added to nickel in the manufacture of an alloy such as one containing 75% nickel and 25% chromium, it will be found that the metallic chromium is difficult to fuse as well as being very expensive, and if the alloy is formed in an electric furnace the carbon content will be raised, which is extremely undesirable.

By my invention I have evolved a process whereby these high melting point metals may readily be obtained in a form adapted for use in making alloys, which is based upon the discovery that the fluorine compounds of these metals can be reduced with extraordinary ease, and that if the oxides are mixed with a substance adapted to generate fluorine at reducing temperatures there appears to be some interaction of the fluorine with the oxide which permits the oxide to be readily reduced. The fluorine compound used may be one of which the resulting stable ingredients will go off with the slag or will enter

55

60

65

70

75

80

85

90

95

100

into the metal product such for example as a fluoride of the metal to be reduced or of some other high melting point metal or a double fluoride of such a metal, or a some-  
 5 what different type of fluoride such as sodium fluoride. It is also advisable to have a re-  
 ducing agent such as silicon or aluminum present (which appears to combine with some of the fluorine) and I also find it advan-  
 10 tageous to incorporate some lime in the mixture which appears to take up excess fluorine, forming fluorspar which keeps the slag fluid, also helping to prevent the escape of fluorine which would tend to poison the atmosphere.  
 15 Thus far my researches have shown only the empirical results, and I am unable to give any satisfactory explanation of what transpires, but apparently the fluorine acts in the nature of a catalyst to aid in the re-  
 20 duction of the oxide.

In any event, the fluorine compounds (such for example as chromium fluoride) act in a very different matter from the oxides or any other compound with which I have worked, 25 for instead of the reduction being slow and only partial, it is almost instantaneous and is complete. Where the metal is in whole or in part in the form of the oxide mixed with the fluorine compound (which may be a com-  
 30 pound of the same metal or some other compound) the reduction is somewhat less rapid, but still is quantitative provided sufficient fluorine is present, as for example in the case of a mixture comprising approximately three 35 parts by weight of chromite and 1 part of chromic fluoride. This relationship is one which I have found satisfactory but is not given as establishing a limit.

As regards the reducing agent, I find that 40 silicon is somewhat more efficient than aluminum. This is apparently due to the fact that silicon and fluorine combine to form a gas which in turn may react on the oxide. In either case, the amount of reducing sub-  
 45 stance that need be used can be calculated, so that there will not be a residue to go over into the resulting product.

The compounds of the metal to be reduced are preferably finely ground and mixed with 50 the reducing agent and with lime and then thrown on a hot slag which may cover a melted metal such as iron with which the high melting point metal is to be alloyed, or may cover a bath of the metal which is 55 being reduced or a ferro compound thereof. The reduced metal will trickle through the slag into the bath and will not be reoxidized by the air.

For carrying on the process, the furnace 60 should be lined with a refractory material that is not readily acted upon by fluorine. I find a lining of magnesite and a roof of chromite can be used, whereas, if silica brick or fire brick is used for the lining, they will 65 melt away very rapidly.

My invention enables me to make chrom-  
 ium alloys with iron or nickel bases such as 70 rustless iron or steel or alloys of the well-known nichrome type at a very low cost.

Alloys containing zirconium have hereto-  
 fore been very difficult to produce and as 75 far as I know it has never been possible to produce a ferro-zirconium having a low silicon content. Zirconium is a valuable alloy in steel, but its use remains undeveloped due to the fact that it has always been accompanied by silicon which has befogged and complicat-  
 ed the true effects of the zirconium in iron. 80

Tantalum is a very excellent alloying steel 85 but heretofore one could not alloy it with steel without great loss due to oxidation, and the entrapped oxides caused the alloy to be so dirty that the good effects of the tantalum were obscured by mechanical defects.

Titanium also is difficult to get into steel 85 in any but small proportions, because ferro-titanium thrown on the surface oxidizes readily. The carbide is useless for anything except as a degasifier.

Uranium is a very useful element in steel 90 but very difficult to incorporate because it oxidizes so readily.

Vanadium is used to a considerable extent 95 in making ferrous alloys, but its use has been restricted due to the high cost of ferro-vana-  
 dium. By my process the vanadium and the 100 other alloying metals referred to can be incor-  
 porated into the bath without difficulty. For example, in the case of vanadium, the simple fluoride  $VF_3$  may be used, whereas, in other instances such as with tantalum or titanium, it may be found more convenient to use a double fluoride.

For the purposes of illustration I will de-  
 scribe my process as applied to the use of 105 chromium, but it is to be understood that the same procedure may be applied to other high melting point metals such as are used for making alloys.

In the manufacture of an alloy of the ni-  
 chrome type containing for example 75% 110 nickel and 25% chromium, the nickel is first melted down, preferably in an electric fur-  
 nace. Sufficient slag is used to protect the metal from oxidation and the molten mass 115 is degasified by the usual methods. Ordinarily it will not be necessary to replace the original slag.

The required amount of chromium fluoride 120 (see examples below) is mixed with lime, and if desired, a small amount of aluminum or silicon can be included. These materials are thoroughly mixed together and then thrown on the slag covering the molten nickel, preferably with the arc turned on. The 125 reaction takes place almost instantly, the additions fusing almost as quickly as they touch the slag. The chromium which is converted quantitatively to melted metal passes down through the slag and mixes with the nickel. 130

As soon as all action stops, the furnace can be tilted and the heat poured. The amount of aluminum or silicon used must be kept low unless it is desired to have one of these substances in the finished alloy. The following are illustrative proportions which I have used successfully:

*Example 1.*—Nickel 80 ounces,  $\text{CrF}_3$  51 ounces, lime 24 ounces, aluminum 3 ounces.

10 The weight of the poured ingot was 106 ounces which on analysis showed 75% nickel and 25% chromium, the conversion of the chromium fluoride having been complete.

15 *Example 2.*—A similar run, but omitting the aluminum, was found to give substantially identical results.

*Example 3.*—Nickel 80 ounces,  $\text{CrF}_3$  51 ounces, lime 24 ounces, silicon 8 ounces.

20 The weight of the poured ingot was 110 ounces and showed the following analysis: Nickel 71.45%, chromium 24.9%, silicon 3.65%.

Here, as before, the chromium conversion was complete.

25 In the manufacture of rustless heat and acid resisting, or stable surface iron or steel there are two procedures which can be conveniently followed: In one case the chromium is all added as chromium fluoride, whereas, in the other case the combination of chromium fluoride and chromite is used. In either case I find carbon is not an advantageous reducing agent to use, for it is slow and wasteful and tends to raise the carbon content of 35 the melt.

30 The use of chromium fluoride alone may be illustrated by the case of the production of an iron alloy containing 15 or more percent of chromium: The iron is melted down in an electric furnace and the carbon is removed by the use of mill scale or iron ore. The slag is removed and replaced by a clean lime slag. The bath is degasified with ingot aluminum held under the metal and by shot aluminum 45 on the slag. To the above slag which will contain calcium oxide together with some aluminum oxide, I add the chromium fluoride mixture prepared similarly to the examples previously described, or as shown by the following examples:

40 *Example 4.*—Iron 80 ounces,  $\text{CrF}_3$  24 ounces, lime 12 ounces.

45 The reduction of chromium was complete and the slag produced was very white. The total procedure occupied but a very short time. The iron was melted in an electric furnace of the arc type in 15 minutes, degasified in 5 minutes, using 2 ounces of aluminum as shot on the slag, and the mixture of chromium fluoride and other ingredients was added to the surface of the molten metal slag in 2 minutes. The mixture fused practically as soon as it was thrown on but the mass was allowed to stand for 5 minutes before pouring. The 55 ingot weighed 98 ounces and due to the

amount of aluminum that was employed, a substantial amount was found in the product as shown by the following analysis: chromium 12.35%, aluminum 5.6%, carbon .02%, iron balance.

50 Another test melt comprised the following:

*Example 5.*—Iron 80 ounces,  $\text{CrF}_3$  8 ounces, lime 8 ounces, aluminum 2 ounces.

The ingredients were handled exactly as in the previous example. The poured ingot 75 weighed 84 ounces and showed an approximate analysis of: chromium 4.76%, aluminum 0%, carbon .01%, iron balance.

In this case it is to be noted that no aluminum went into the finished product but the conversion of chromium was complete. By increasing the amount of chromium fluoride used, the percentage of chromium may be increased to any desired point, so that if the melted metal in the bath is fused chromium, 85 substantially 100% chromium can be obtained.

If an addition of zirconium, vanadium, tantalum, titanium, uranium or the like is required, a fluoride or double fluoride of such metal can be mixed with the chromium fluoride and the conversion can be conducted in substantially the same way; or these materials can be used alone or mixed together without the use of any chromium fluoride.

90 The examples are set forth in terms of small quantities which were used for the purpose of simplifying measurements and analyses; but my experience has shown that substantially the same conditions will hold good 100 for large batches.

I have described these examples as conducted in the electric arc type of furnace but other types of furnace can be used and the process is particularly adapted to open hearth 105 practice. It is to be understood that the ingredients added to the slag can be preheated if desired to a point below that at which fluorine is liberated and if desired powdered additions can be briquetted to facilitate handling.

110 Where fluoride and oxide are used together and where it is desired to keep the silicon or aluminum content very low, the theoretical amount of silicon or aluminum to be used 115 may be calculated as follows:

Approximately one-fifth as much silicon or aluminum or both should be used to take care of the chromium fluoride, while 18% of the weight of chromite in silicon or 21% of 120 the weight of chromite in aluminum should also be included.

When a fluoride (of the metal or some other fluoride) is used in conjunction with the metallic oxide, it is apparent that the 125 fluorine has some effect on the oxide, for the reduction of the oxide will take place with great rapidity and can be completed with only the theoretical amount of reducing agent present. The following are examples 130

of the combined use of chromium fluoride and chromite:

*Example 6.*—Iron 80 ounces,  $\text{CrF}_3$  16 ounces, chromite 48 ounces, lime 12 ounces, 80% ferrosilicon 12 ounces.

The iron was melted down in 15 minutes. The melt was degassed with one ounce of shot aluminum thrown on the lime slag. A mixture of powdered chromium fluoride, chromite, lime and ferro-silicon which had previously been well mixed, was thrown on the slag with the arc turned on. It took 6 minutes to make this addition but the mixture fused almost as quickly as it was added. The heat was allowed to stand with the arc on for ten minutes, though the action appeared to end in about five minutes after the last addition was made. The heat was poured and the ingot resulting weighed 110 ounces, which was the full theoretical weight. The chromite was found to be entirely reduced and the chromium fluoride to be entirely converted. The approximate analysis of this heat was: chromium 24.20%, carbon .01%, iron balance.

A similar heat was made using aluminum in place of silicon with identical results being obtained, though the action was not quite as rapid.

In another case a run was made to check up the accuracy of the process. The ingredients used were as follows:

*Example 7.*—Iron 80 ounces,  $\text{CrF}_3$  6 ounces, chromite 16 ounces, lime 6 ounces, 80% ferro-silicon 7 ounces.

If one disregards the excess silicon, the theoretical weight of the finished ingot will be 93 ounces. However, it can be calculated that there has been used a theoretical excess of silicon approximating 1.5 ounces. When the heat was finished and poured it was found that the finished ingot weighed 94.5 ounces, giving exactly the theoretical results. The approximate analysis of the ingot was: chromium 8.75%, silicon 5.25%, carbon .01%, iron balance.

If one desires to make ferro-chromium instead of producing the alloy directly, this can be done either by converting chromium fluoride in a large quantity over a bath containing a relatively small amount of iron or the chromite and chromium fluoride can be treated jointly, as shown by the following example:

*Example 8.*—Iron 4 ounces,  $\text{CrF}_3$  48 ounces, chromite 144 ounces, lime 24 ounces, 80% ferro-silicon 48 ounces (Fe 9.6 ounces).

This composition gave an ingot weighing 105 ounces (which is almost exactly the theoretical weight) containing approximately 70% chromium and 30% iron.

For the manufacture of ferro-chromium I prefer to use a multiple electrode arc furnace having a roof instead of the open type arc furnace. However, in view of the speed

of the reaction and the extremely liquid type of slag an electric type arc furnace of the reducing type can be used or an open hearth furnace can be employed, particularly when the chromium ingredients are preheated.

Heats made by my process can have any desired ferro alloys added to them or the initial bath may be rich in one or more of the elements. While I prefer to use an initial bath which will prevent the high melting point metal from becoming oxidized, it may be possible to omit this under certain conditions.

While the foregoing examples are restricted to chromium and to chromium compounds of fluorine, it is to be understood that they are equally applicable to other high melting point alloying metals, though of course some difference in relative amounts of ingredients might have to be made (due to differences in valences, molecular weights and the like) as anyone skilled in the art will readily understand. Also in place of the fluorine compound of the metal other fluorine compounds such for example as sodium fluoride can be used to supply fluorine to react with the oxide. Such fluorine compound should be one which will decompose at or below the melting point of the metal but will not decompose at relatively low temperatures, as otherwise the fluorine may escape as a gas before the metallic compound reaches the reducing temperature.

What I claim is:

1. The process of reducing a compound of a high melting point metal of the type used in making ferrous alloys, which comprises the step of throwing on a hot fused slag a mass comprising a fluorine compound of such metal.

2. The process of reducing a compound of a high melting point metal of the type used in making ferrous alloys which comprises the step of throwing on a hot melted slag a mixture comprising an oxide of such a metal, a fluorine compound of such a metal and a reducing agent.

3. The process of producing ferrous alloys which comprises the step of forming a bath of molten ferrous metal with a slag on the surface and adding to such slag a finely divided mass comprising a fluorine compound of an alloying metal.

4. The process of producing chromium alloys which comprises the steps of forming a melted bath of metal with a slag on the surface and adding to such slag a mass comprising chromite, chromium fluoride and a reducing agent.

PERCY A. E. ARMSTRONG.

70

75

80

85

90

95

100

105

110

115

120

125

130